

March 26, 1968

R. STUBBINGS

3,374,496

METHOD OF LASTING LEATHER UPPERS

Filed Nov. 3, 1965

2 Sheets-Sheet 1



FIG. 1

INVENTOR.

Robert Stubbings  
BY  
Kenway, Jenney & Hildreth  
Attorneys

March 26, 1968

R. STUBBINGS

3,374,496

METHOD OF LASTING LEATHER UPPERS

Filed Nov. 3, 1965

2 Sheets-Sheet 2

ROOM MOISTURE, SHRUNKEN AT 375°F. FOR VARIOUS TIMES,  
10 MIN. COOLING, RELEASE.



FIG. 2



FIG. 3

INVENTOR.

*Robert Stubbings*

BY

*Kenway, Jenney & Hildreth  
Attorneys*

## 1

3,374,496

**METHOD OF LASTING LEATHER UPPERS**  
Robert Stubbs, 7721 N. Regent Road,  
Milwaukee, Wis. 53217  
Filed Nov. 3, 1965, Ser. No. 506,250  
7 Claims. (Cl. 12—145)

**ABSTRACT OF THE DISCLOSURE**

Process of shoemaking wherein a leather upper is assembled on a last without substantial stretching so that the upper assumes the general contour of the last, drying the unlasted upper (if not already moisture free when assembled on the last and heating the upper to between 250° and 450° F. to shrink the upper and cause it to last itself.

My invention relates to shoemaking and comprises a novel method of lasting leather shoes.

Heretofore it has been almost universal practice to assemble an upper on a last to which an insole has been secured. Then the assembled upper is pulled over the last by machine, the lower margins of the upper being tacked temporarily to the insole. Subsequently the sides, the toe, and the heel seat portions of the upper are tightly pulled over the last and their overlasted margins permanently secured to the insole.

Relatively recently there have been developments designed to increase the faithfulness with which the upper conforms to the shape of the last and to decrease the time the upper must remain on the last in order to retain permanently the desired shape. In general these new developments are referred to as "heat setting" and involve subjecting the shoe, while still on the last, to heat, with or without added moisture, at temperatures ranging up to about 250° F.

I have discovered that if an upper of relatively dry leather is assembled loosely upon a last and then subjected to a temperature between 250° F. and 450° F., the heat will cause the upper to shrink and actually last itself in a few minutes. Moreover, the shoe so made will retain the shape of the last to a degree not hitherto achieved. The last can be removed as soon as the heating step is over, since the leather of the upper will have taken a permanent set.

In addition to the marked increase in the quality of the finished shoe, the process of my invention has important economic advantages. The relatively costly lasting machines can be eliminated, together with many lasting operations requiring highly skilled workers. Hence shoes of the finest quality can be produced at reduced cost.

Other features of my invention will be more readily understood and appreciated from the following detailed description of a preferred embodiment thereof, selected for purposes of illustration, together with the accompanying drawings, in which:

FIG. 1 is a graphical representation of the shape retention ("set"), of leather uppers given various kinds of treatment,

FIG. 2 is a graphical representation showing the effect of varying the time of treatment, and

FIG. 3 is a graphical representation showing the effect of different temperatures as well as the difference in treating loosely lasted and tightly lasted shoes.

In conventional lasting the leather is stretched from about 15% to 35% in area, as the result of the action of the lasting pincers in gripping and pulling the upper about the last. If such a shoe is then subjected to moist heat at about 250° F. and then removed from the last, the shoe will retain about 70% to 80% of the shape set. For a discussion of the measurement techniques I refer to a

## 2

paper by Butlin (J.S.L.T.C., 47, 3, 1963) and my paper in the January issue of the Technical Journal of the National Footwear Manufacturers Association, vol. 3, No. 1, p. 23 et seq.

It will first be necessary to define some of the terminology involved. I use the term "tightly lasted" to refer to conventional lasting in the course of which the percentage of stretch of a given area of the upper will be from about 15% to 35%. By "loosely lasted" I mean a lasting process in which a given area of the leather upper will be stretched from zero to about 10% so that the upper loosely assumes the general contour of the last. The determination of the amount of such stretch may most conveniently be made by employing the grid system disclosed in detail in my paper cited in the foregoing paragraph. Briefly, a grid pattern of .1" is printed on the flat leather parts of the shoe before they are stitched to form an upper. After the printed upper has been lasted, measurements may be made of the distortion of the pattern caused by the stretching of the leather during the lasting.

In FIG. 1 there is graphically presented the results of experiments during which upper leather was subjected to treatment at various temperatures, for various times, using leather having different moisture contents. The curves show the loss and percentage set up to 100 hours after the last has been removed. It will be seen that the optimum set is achieved when the upper is fairly dry (12% moisture), the stretch is zero, and the upper has been subjected to 375° F. for three minutes. The next most favorable result is achieved with an upper having from 12% to 30% moisture, loosely lasted and subjected to 375° F. for five or ten minutes. In both examples, the temperature and time are sufficient to completely dry the upper so that it is moisture free and thereafter shrink the upper to cause it to last itself. The same figure reveals that a tightly lasted shoe will not hold its set, regardless of other conditions of treatment, in any way comparable to the set retention exhibited by loosely lasted shoes subjected to heat treatment.

FIG. 2 shows graphically the effects produced by varying the duration of the heating step from thirty seconds to five minutes and reveals that the optimum period is from three to five minutes, provided that the upper is relatively dry to start with.

Other tests show that the shrinkage takes place when the upper has been dried so that its moisture content is approximately 12% to 15%. If an upper having, say, 30% moisture is subjected to a temperature between 250° F. and 475° F., it will be found that there is an appreciable period before the shrinkage takes place; during this period the leather loses moisture until its moisture content has been reduced to from 12% to 15%. As soon as that condition is reached, the shrinkage takes place in less than three minutes. If the leather is wringing wet, having a moisture content appreciably greater than 35%, the result of treatment at the temperatures here involved will be to ruin the leather. It is therefore an essential condition for successful operation of the process of my invention that the leather have a moisture content not greater than about 35%.

In FIG. 3 there is a graphic representation of the results of tests made to determine the effect of varying temperatures, and the curves demonstrate that a loosely lasted upper treated at 265° F. for five minutes will retain its set very much more faithfully than either tightly or loosely lasted uppers treated at lower temperatures. Various types of upper leather are available on the market, and there is probably for each type a threshold temperature below which the phenomenon here utilized will not take place. In general, however, it is safe to use 250° F. as a practical lower limit.

Of course, if the temperature is too high, the leather will be burned or otherwise adversely affected. Here again I do not believe there is a critical upper limit applicable to all types of leathers. As a practical matter, however, 450° F. appears to be about as high as it is safe to go. Obviously it is better practice to operate well within the extremes, and a temperature of 375° F. is therefore recommended. It should be stated that the upper limit for the operating temperature is governed to some extent by the moisture content of the leather upper being treated. If the moisture content is in the neighborhood of 30%, it is wise to operate at the lower portion of the temperature range; if the leather has a moisture content close to the low end (12% to 15%), the treatment may be carried out at a temperature approaching the high end of the margin.

I have conducted experiments to determine whether or not it is essential that the lasted upper be cooled, after the heat treatment has been carried out, but the results showed that a cooling step is technically unnecessary, although for practical reasons it is desirable that the upper be permitted to cool down approximately to room temperature before the last is removed.

Those skilled in the art will immediately understand that the process of my invention is based on two principles which run counter to commonly accepted shoemaking practice. The temperature range of from 250° F. to 450° F. is very much higher than it has been thought safe to employ. Also, it has been almost universal practice to mull uppers prior to lasting, since an increase in moisture content renders leather easier to last. In this connection it should be pointed out that in addition to eliminating conventional lasting processes and equipment, the process of my invention also eliminates the mulling step.

While it is preferable that the shoe be loosely lasted, the beneficial results of the process of my invention can be secured by other means. Generally this involves providing means whereby the upper can shrink back to zero percent area stretch. For example, a shoe may be lasted in conventional manner, the last removed, and another last inserted, the second last being a size smaller than the first last; the re-lasted shoe is then heat shrunk in accordance with my invention. Alternatively, it might be possible to provide a last fitted with means for reducing its volume after lasting and before the heat treatment is utilized.

I have found that the dry heat shrinkage process of my invention in no way adversely affects the quality of the leather. There is no change in its flexibility, strength, stiffness, or grain pattern.

Those skilled in the art will readily understand and

appreciate the many variations which may be utilized in carrying out the process of my invention, the scope of which is measured by the appended claims.

I claim:

- 5 1. The process of shoemaking comprising the steps of assembling a leather upper having a moisture content on a last without substantial stretching so that the upper assumes the general contour of the last, drying the unlasted upper while so assembled on the last by subjecting the same to heat between 250° and 450° F. for a period of time sufficient to remove substantially all moisture from the upper, and continuing the heating within said temperature range to cause the upper to shrink and last itself, and thereafter removing the upper from the last.
- 10 2. The process as set forth in claim 1 wherein the temperature is about 375°.
- 15 3. The process as set forth in claim 2 wherein the moisture content of the upper before it is placed on the last is about 12%.
- 20 4. The process as set forth in claim 3 wherein the overall heating period is about 3 minutes.
- 25 5. The process of shoemaking comprising the steps of assembling a moisture-free leather upper on a last without substantial stretching so that the upper assumes the general contour of the last, subjecting the unlasted upper while so assembled on the last to heat at a temperature between 250° to 450° F. to cause the upper to shrink and last itself, and thereafter removing the upper from the last.
- 30 6. The process as set forth in claim 5 wherein the temperature is about 375° F.
- 35 7. The process of shoemaking comprising the steps of assembling a leather upper having a moisture content of about 12% to 30% on a last without substantial stretching so that the upper assumes the general contour of the last, drying the unlasted upper while so assembled on the last by subjecting the same to heat at about 375° F. for a period of time sufficient to remove substantially all moisture from the upper, and continuing the heating at
- 40 40 said temperature to cause the upper to shrink and last itself, the overall heating period being from about 5 to 10 minutes, and thereafter removing the upper from the last.

#### References Cited

#### UNITED STATES PATENTS

|            |        |           |       |        |
|------------|--------|-----------|-------|--------|
| Re. 25,411 | 7/1963 | Bromfield | ----- | 12—142 |
| 2,973,530  | 3/1961 | Bromfield | ----- | 12—142 |
| 3,176,333  | 4/1965 | Maeser    | ----- | 12—142 |
| 3,237,227  | 3/1966 | Bromfield | ----- | 12—1 X |

PATRICK D. LAWSON, Primary Examiner.